

## United States Patent Office

2,711,974

Patented June 28, 1955

## 1

2,711,974

## COATING FOR METALS

Arthur H. Happe, Detroit, Mich., assignor of one-half to  
Herman A. Sperlich, Detroit, Mich.

No Drawing. Application December 8, 1951,  
Serial No. 260,765

3 Claims. (Cl. 117—127)

The present invention relates to the coating of metals to protect them against corrosion under the influence of moist or dry heat, and to make them resistant to chemical action and to erosion.

Among the objects of the invention is to provide a coating applicable to steels, aluminum, and other metals now used and proposed to be used for the construction of engine parts, plane parts, and other articles.

Another object is to provide a coating which shall have good adherence under severe conditions such as violent temperature changes, distortion, high temperatures, etc.

Another object is to provide a coating which may be applied as a thin coating and therefore less subject to chipping.

With these and other objects readily occurring to those skilled in the art, the invention consists broadly in the application by dipping, spraying or otherwise to the metal object a mixture of silicates and metallic oxides in a water vehicle, allowing to dry and then baking at a relatively low temperature.

A composition which has given excellent results consists of the following ingredients in the proportions indicated:

| Percent by weight                                                                          |    |
|--------------------------------------------------------------------------------------------|----|
| 1.290 sp. gr. water solution of <u>sodium silicate</u> having a <u>high sodium content</u> | 50 |
| Metal oxides                                                                               | 30 |
| Exfoliated vermiculite                                                                     | 10 |
| Kaolin                                                                                     | 10 |

The metal oxides are preferably about equal parts of nickel and cobalt oxides, but good results have been obtained using titanium or chromium for part or all of the nickel and cobalt oxide.

## 2

These materials are thoroughly mixed and ground together in a suitable mill and the result applied to the thoroughly cleaned metal. After drying, the coated metal is placed in a suitable oven and brought to a minimum temperature of 750 to 800° F. It is then ready for use.

The above proportions admit of some variation without material detriment. For example, the percentage of each of the metallic oxides may be varied to from 12-17% with a corresponding change of the other from 17-12% while the amounts of exfoliated vermiculite and kaolin may be increased or decreased one or two per cent. The exfoliated vermiculite is preferably the product found on the market under the trade name of "Zonolite."

In the use of the coating, it has been successfully applied to steels, surface treated steels, enameling iron, aluminum, magnesium, magnesium alloys, titanium, molybdenum, and alloys of the latter two.

## I claim:

1. A coating composition for metals consisting of  
20 1.290 sp. gr. water solution of sodium silicate having a high sodium content----- 50% by weight  
Cobalt oxide----- 15% by weight  
Nickel oxide----- 15% by weight  
Exfoliated vermiculite----- 10% by weight  
25 Kaolin ----- 10% by weight

2. A coating composition for metals consisting of  
1.290 sp. gr. water solution of sodium silicate having a high sodium content----- 50% by weight  
Cobalt oxide----- 12-17% by weight  
30 Nickel oxide----- 17-12% by weight  
Exfoliated vermiculite----- 10% by weight  
Kaolin ----- 10% by weight

3. The process of coating metals which consists in  
35 applying thereto a thin layer of an intimate mixture of  
1.290 sp. gr. water solution of sodium silicate having a high sodium content----- 50% by weight  
Cobalt oxide----- 15% by weight  
Nickel oxide----- 15% by weight  
40 Exfoliated vermiculite----- 10% by weight  
Kaolin ----- 10% by weight  
and heating to a temperature of at least 750-800° F.

## References Cited in the file of this patent

- 45 UNITED STATES PATENTS  
1,921,468 Jack ----- Aug. 8, 1933  
2,364,436 Frisch ----- Dec. 5, 1944  
2,462,763 Nightingall ----- Feb. 22, 1949